

May 31, 1938.

R. C. MERRILL

2,119,238

## PRECIOUS METALS ALLOYING APPARATUS

Filed Feb. 14, 1938

2 Sheets-Sheet 1



May 31, 1938.

R. C. MERRILL

2,119,238

PRECIOUS METALS ALLOYING APPARATUS

Filed Feb. 14, 1938

2 Sheets-Sheet 2

Fig. 4



Fig. 5



Fig. 8



Fig. 7



Fig. 11 Fig. 12



Fig. 9

INVENTOR,  
Richard C. Merrill.  
BY David E. Lain,  
ATTORNEY.

## UNITED STATES PATENT OFFICE

2,119,238

## PRECIOUS METALS ALLOYING APPARATUS

Richard C. Merrill, Cave Junction, Oreg.

Application February 14, 1938, Serial No. 190,452

5 Claims. (Cl. 266—34)

Precious metals, when occurring in their native state, may be completely extracted from their ores by alloying with lead. For this purpose the ores are pulverized finely and mixed with molten lead after which, the finely comminuted rock, "sand", is removed from the alloy and then the precious metals are separated from the lead.

My invention has for an object to thoroughly mix the pulverized ore with molten lead.

Another object of my invention is to completely separate the sand from the metal alloy.

Another object of my invention is to provide for the free dripping of the alloy from the sand during the process of the separation thereof.

Another object of my invention is to provide a vessel in which the said separation may occur wherein the rising mixture of sand and alloy enters increasing areas.

Another object of my invention is to provide the said vessel and stirring appurtenances therein in and among which the said mixture may rise into increasing areas without having enlarged the diameter of the vessel as its top is approached.

Other objects of my invention will appear as the description proceeds.

My invention is illustrated in the two sheets of accompanying drawings, which form a part of this specification, in which Figure 1 is a side elevation of my precious-metals alloying apparatus in section on a longitudinal, vertical, medial plane, Fig. 2 is a sectional view of the pipe of the apparatus on a transverse plane through the line 2—2 of Fig. 1, Fig. 3 is a sectional view of the said pipe on a transverse plane on the line 3—3 of Fig. 1, Fig. 4 is a top plan view of Fig. 1 from which the major portion of the pipe has been broken away, Fig. 5 is the front end elevation view of the apparatus, Fig. 6 is a top plan view of the bowl on a horizontal plane through the line 6—6, Fig. 7 is a side elevation of one of the three similar stirring and elevating paddles segregated, Fig. 8 is a top plan view of Fig. 7, Fig. 9 is a bottom plan view of Fig. 7, Fig. 10 is an edge elevation of Fig. 7 limited to the said edge, Fig. 11 is a side elevation of an optional shape of stirring paddle, and Fig. 12 is an edge view of Fig. 11.

Throughout the specification, similar designating characters refer to similar parts. Certain parts are broken away.

With more particular reference to designated parts: The bowl 13 is a vertically disposed hollow cylinder with a closed rounded bottom, open

top and overflow lip 13a. Connected with the bottom of the bowl and extended horizontally is the pipe 14, with removably fastened cover 14a, 14b, closed outer end 16, an upwardly extended chamber 17 at its outer end closed by the removably fastened cover 18 and an upwardly extended receiving tube 19 on the cover 14a. A centrally-disposed stationary shaft 15 has its bottom end fastened in the bottom of the bowl 13 and extends above the top of the bowl.

A vertical shaft 20 is mounted for revolution in a bearing at the outer end of the pipe 14 on the bottom thereof and in a bearing on the pipe cover 18 above which it is extended and has fastened on its lower end, within the pipe, the bevel gear 21 and, on its upper end, above the pipe, the bevel gear 22. On a bracket 24a the bearing 24 is fastened to mount for revolution the drive shaft 23 which has the bevel gear 25 fastened thereon meshing with the gear 22. The bracket 24a is fastened on the pipe cover 18. The bearings 26 and 27 are fastened to hangers from the inside of the pipe cover 14a and mount the shaft 28 for revolution within the pipe 14 disposed parallel therewith and above the center thereof. On the outer end of the shaft 28 is fastened the bevel gear 31 meshed with the gear 21. The bevel gears 21, 22, 25, and 31 are conventionally drawn. The construction provides for the shaft 28 to be driven by the shaft 23. There are five two-blade propellers 29 shown as fastened, spaced apart, on the shaft 28 and the two-blade propeller 29a fastened on the said shaft near its outer end. On the end of one of the blades of the propeller 29a is fastened the arm 30 extended at right angles therewith. The shaft 28 passes through a hole in the baffle plate 32 which is disposed adjacent the gear 31 and fastened to the bottom side of the pipe cover 14a and its bottom end is spaced from the bottom of the pipe 14. All of the blades of the said propellers are set for forcing a movement of any contents of the pipe 14 from its outer end toward the bowl 13 when the shaft 28 is revolved clockwise as viewed from its outer end. The shaft 28 is disposed to revolve the ends of the propeller blades adjacent the cover 14a and spaced from the bottom of the pipe 14. The arm 30 is disposed to pass near and beneath the inner end of the receiving tube 19 as the shaft 28 revolves.

Within the cylindrical bowl 13 is disposed the hollow cylindrical intruding element 33 having the conical bottom end 34 and an interior flanged open upper end closable by the cover 35 and 55

mounted for revolution on the stationary shaft 15. The cover 35 is fastened to the shaft 15 by the set screw 37 to prevent the same from revolving and may be fastened to the flange of the element 33 by the cap screws 36, 36; which are shown in dotted lines. When retained by the screws 36 the element 33 can not revolve on the shaft 15, but when the said screws are removed from the cover and flange, the element 33 is free to revolve on the shaft 15. The vent hole 35<sup>a</sup> provides against the accumulation of pressure within the element 33. The element 33 is disposed within the bowl 13 to provide the annular space 48 between the bowl and element.

15 The annular disc 38 is mounted for revolution on the shaft 15 above the cover 35 and has the centrally disposed bevel gear 39 fastened on its top surface. The bracket 41 is fastened on the top end of the shaft 15 and has the horizontal bearing 40 in which is mounted the shaft 42 for revolution. On the inner end of the shaft 42 is fastened the bevel gear 44 meshing with the gear 39. The gears 39 and 44 are conventionally drawn. The construction provides for the revolution of 25 the disc 38 by the shaft 42. Beneath the disc 38 are three dependent paddles 43, 43, 43 fastened to the disc with two studs 45, 45, on the upper end of each paddle, which are extended through holes in the disc and retained in place by nuts thereon. 30 The paddles 43 are disposed within the annular space 48 and transversely arcuate concentric with the said space. These paddles extend from the bottom of the disc 38 to a point within the bowl 13 adjacent the base of the conical bottom end 35 of the element 33. The shaft 42 is turned to revolve the disc 38 in a clockwise direction, as viewed from the top thereof, and the rear edges of the paddles 43 are vertically disposed while the forward edges of the paddles extend diagonally downward and forward as shown at 43<sup>c</sup>. 40 This construction provides for the bottom ends 43<sup>a</sup> of the paddles being wider than the top ends thereof. There are spaced vertical grooves 43<sup>b</sup> in each side of each of the paddles 43 and a groove 45 43<sup>c</sup> in the rear edge of each of the said paddles. These grooves extend upward no farther than the level of the overflow lip 13<sup>a</sup> in the top edge of the bowl.

When the character of the ore makes the 50 straight plane paddles 46, 47 preferable to the more complicated structure above explained with reference to paddles 43, they may be used to replace the latter.

In operation: Assume that the lower part of 55 the apparatus is filled with molten lead about to the level of line a—a of Figs. 1 and 5; that the apparatus is disposed in a heated furnace capable of maintaining the said lead at a temperature of about 1000° F.; that the paddles 43 are being 60 revolved in the annular space 48; that the propellers 29, 29<sup>a</sup> are revolving in the pipe 14, and that finely comminuted ore is being poured into the top of receiving tube 19. Then the ore will tend to float on the top of the molten lead but 65 will be carried beneath the surface of the lead and mixed therewith by the arm 30 and the blades of the propellers 29, 29<sup>a</sup> revolving in the pipe 14. The mixture of ore and lead in the pipe 14 will be shoved toward the bowl 13 by the propellers and, 70 arriving in the bottom of the bowl, it will rise in the annular space 48 to be carried around therein by the revolving paddles 43. With the cap screws 36 in place, as shown in dotted lines in Fig. 1, the element will remain stationary. This 75 is desirable when alloying some ores; but, or-

dinarily, I prefer to not use the said cap screws and leave the said element free to revolve under the frictional impulse of the ore and lead revolving in the annular space 48. The front edges 43<sup>c</sup> of the paddles, moving forward in the annular space 48, will tend to lift upward on the ore and aid the propelling action of the propellers 29, 29<sup>a</sup> in the pipe 14 to shove the ore up and out over the lip 33<sup>a</sup>.

The greater width of the paddles 43 at the 10 bottom than at the top thereof reduces the available space for ore and lead in the bottom of the annular space 48 as compared with the said space at the top of the bowl. That is, the rising column in the annular space enters areas of greater 15 capacity as it moves upward, thus diminishing the tendency of the tenacious material to solidify and clog the space in which it is being agitated by the paddles. It is desired to entirely separate the sand from the alloy during the movement of the 20 material from the upper surface of the lead in the bottom of the bowl to the top of the bowl. This is aided by maintaining the temperature within the annular space 48 to the very top of the 25 bowl. It is further aided by the grooves 43<sup>b</sup>, 43<sup>c</sup> in the paddles 43. As these paddles are forced 30 forward in the annular space among the mixture of sand and alloy, with much of the alloy firmly adhering to the sand, these grooves provide small vertical conduits from near the top of the 35 bowl to the lead in the bottom thereof through which alloy, which is adhering to the sand but which tends to leave the same when contacting with the hot metal paddles, may freely flow to the said metal in the bottom of the bowl. In this way the sand may reach the top of the bowl and flow over the lip thereof quite entirely free from the 40 said metallic alloy.

When it is desired to "clean up", feeding in of the crushed ore ceases, but otherwise the machine 40 operates as described till sand no longer flows over the bowl. Then power is shut off, the disc 38 with top gears and bottom paddles are removed, as also are the cover 35 and element 33, exposing the bowl 45 for convenient removal of its contents. The sand and sand with lead attached are removed and reserved for again passing through the machine. Then all of the molten alloy is removed and treated for separating the precious metals 50 contained therein. The lead remaining, after the removal of other metals of the alloy, is returned to the machine for further use.

Having thus disclosed my invention, what I 55 claim as new therein and desire to secure by Letters Patent is,—

1. Apparatus of the kind described including, a cylindrical bowl, a substantially horizontally disposed pipe having its outer end closed and its inner end connected with the bottom of the said bowl and having a portion of its upper part removably fastened thereon as a cover, a receiving tube connected with the said pipe cover disposed near the said closed end of the pipe, drivable means disposed within the said pipe adapted to mix any pulverous and fluid contents thereof and advance the said contents toward the said bowl, mechanical connections between the said drivable means within the pipe and driving means outside of the pipe adapted to convey driving power to the said drivable means within the pipe, a vertical shaft centrally disposed within the bowl fastened to the bottom thereof, a cylindrical element mounted on the said shaft for revolution within the said bowl providing an intervening annular space, a disc mounted for revolution on the 75

said shaft disposed above the said element, a plurality of paddles fastened to the said disc extended into the said annular space revoluble therein by the revolution of the said disc, and means to revolve the said disc.

5. 2. In apparatus of the kind described, a cylindrical bowl, a substantially horizontally-disposed pipe having its outer end closed and its inner end connected with the said bowl at the bottom thereof and having a portion of its upper part removably fastened to the lower portion thereof as a cover thereon, the bottom portions of the said bowl and pipe being adapted to contain molten lead, a receiving tube connected with the 10 said pipe near the said outer end thereof, aligned bearings within the said pipe suspended from the said cover thereof, a shaft mounted for revolution in the said bearings longitudinally in the said pipe, a plurality of mixing and propelling blades fastened on the said shaft to revolve therewith, an external driving shaft mounted for revolution on the said closed end of the pipe, driving connections between the said external shaft and the said pipe shaft to revolve the pipe shaft by the driving shaft, a centrally-disposed vertical shaft in the said bowl fastened to the bottom thereof, a cylindrical intruding element mounted on the said bowl shaft for revolution within the bowl providing an annular space 15 between the element and bowl, a disc mounted for revolution on the said bowl shaft above the said bowl and intruding element, stirring paddles fastened to the said disc and extended into the said annular space, and means to revolve the said disc to move the said paddles within the said annular space.

3. Alloying apparatus of the kind described including, a substantially horizontally-disposed pipe having a closed outer end, a receiving tube connected with the said pipe disposed near the said closed pipe end, a longitudinally disposed shaft mounted for revolution in the said pipe, a plurality of mixing and propeller blades fastened on the said shaft to revolve therewith, a horizontal arm fastened on the end of one of the said propeller blades disposed beneath the inner end of the said receiving tube to move in close proximity to the said tube end as the said shaft revolves, a chamber in the said closed end of the pipe extended above the said pipe, a baffle plate fastened transversely in the said pipe between the said tube end and the said end chamber having its bottom end spaced apart from the pipe bottom, a vertical shaft mounted for revolution in

the said end chamber with its upper end extended above the said chamber external thereto, driving connections between the lower end of the said vertical shaft and the outer end of the said pipe shaft, driving connections between the external end of the said vertical shaft and a driving shaft, and the said driving shaft mounted for revolution.

4. Alloying apparatus of the kind described including, a cylindrical bowl, a vertical shaft centrally disposed in the said bowl having its lower end fastened in the bottom thereof, a cylindro-conical intruding element mounted within the bowl on the said shaft free to revolve thereon providing an annular space between the element and the said bowl, and releasable means to prevent the revolution of the said element on the said shaft.

5. In apparatus of the kind described, a cylindrical bowl, a substantially horizontally-disposed pipe having its outer end closed and its inner end connected with the said bowl at the bottom thereof and having a portion of its upper part removably fastened to the lower part thereof as a cover thereon, the bottom portions of the 20 said bowl and pipe being adapted to contain molten lead, a receiving tube connected with the pipe adjacent the closed end thereof, stirring and propelling blades mounted for revolution in the 25 said pipe to mix any pulverous matter with any molten lead in the said pipe and advance them into the said bowl, means external to the pipe mechanically connected with the said blades within the pipe to revolve the blades, a vertical shaft centrally disposed in the said bowl fastened 30 to the bottom of the bowl, a hollow cylindro-conical intruding element mounted in the bowl on the said shaft therein for free revolution providing an annular space between the element and the said bowl, a cover over the said intruding element fastened to the said bowl shaft, removable 35 means to fasten the said cover to the intruding body to prevent its free revolution on the shaft, a disc mounted on the bowl shaft for revolution above the said cover, arcuate stirring paddles 40 wider at the bottoms than at the tops thereof disposed longitudinally in the said annular space having longitudinal grooves in their sides and rear edges fastened to the said disc to be revolved in the annular space with the said grooved 45 edges in the rear, and means to revolve the said disc.

RICHARD C. MERRILL.